

# UNITED STATES PATENT OFFICE.

JOHN H. HALL AND RICHARD D. JORDAN, OF HIGH BRIDGE, NEW JERSEY, ASSIGNEES  
TO TAYLOR-WHARTON IRON AND STEEL COMPANY, OF HIGH BRIDGE, NEW JER-  
SEY, A CORPORATION OF NEW JERSEY.

## MELTING FERROMANGANESE.

1,421,218.

Specification of Letters Patent. Patented June 27, 1922.

No Drawing.

Application filed July 15, 1920. Serial No. 396,414.

To all whom it may concern:

Be it known that we, JOHN H. HALL and RICHARD D. JORDAN, citizens of the United States, residing at High Bridge, in the 5 county of Hunterdon and State of New Jersey, have invented certain new and useful Improvements in Melting Ferromanganese, of which the following is a specification.

10 As indicated, this invention relates to the melting of ferro-manganese.

Generally stated, the objects are to avoid the heretofore usual and undesirable loss of metal, and to simplify and reduce the cost of 15 melting.

According to our invention, the ferro-manganese and appropriate fuel, as for example, coke, are charged in successive layers across the entire area of the cupola, 20 vision being made to avoid the destruction of the cupola lining during the melting operation. As is well known, the oxidation of the ferro-manganese, in melting, produces oxide of iron and oxide of manganese, sub- 25 stantially in the proportions of the iron and manganese as they exist in the ferro-manganese. These oxides attack the lining of the cupola vigorously and if not overcome would soon destroy it. Hence, an essential 30 step of the process is to obviate this condition and this we accomplish through the use of a flux capable of neutralizing the oxides mentioned. A cheap and satisfactory material for this purpose is old clay brick-bats, 35 which are broken up into small sizes and charged in the cupola in appropriate quantities. The cupola lining is thus protected for a longer life, and the resultant fluid slag is tapped from the cupola at desired in- 40 tervals.

A second and important step in the process is the character of the blast pressure, which, according to our invention, is maintained much lower than is usual, in order to 45 avoid appreciable loss of metal. The blast pressure is of the order of from two to eight ounces, and we find that best results ensue with an average blast pressure of about four ounces. Experience has demonstrated that 50 if the pressure is substantially increased, as may be exceptionally necessary for faster melting, the loss of ferro-manganese is increased out of all proportion to the increase of blast pressure.

The third important step in the process 55 is the charging of an excess of metal over the daily requirements of melted material. As the charge in the cupola descends through melting, fresh charges of ferro-manganese and coke are added, so that the cupola is 60 kept constantly full until the end of the day's run. Under the old practice the charging is stopped when the material within the cupola is sufficient in quantity to produce the desired weight of metal, and, hence, a con- 65 siderable loss by weight of ferro-manganese is entailed, owing to the cupola becoming nearly empty before the last metal is tapped. This loss is largely, if not entirely, obviated by the above noted third step in the process, 70 which, as indicated, consists in charging the cupola with a quantity of metal in excess of that required for the day's melt, so that the cupola will be substantially half full after the last metal desired has been tapped. The 75 excess metal may of course be dropped from the cupola in an unmelted condition, separated from the coke after cooling, and re-used for the next melt.

With this process, and with the use of a 80 single cupola it is possible to tap a considerable quantity of ferro-manganese, say about 1100 pounds, from a cupola measuring 30 inches inside diameter, every eighteen or twenty minutes, thereby accomplishing with 85 one cupola what has heretofore been accomplished with five or six movable cupolas. The process therefore tends to a material saving of metal, and also to a material reduction in cost of operation owing to the saving of time and labor in the use of a single cupola as compared with the five or six movable cupolas heretofore necessary to produce 90 the same quantity of material.

Having described our invention, we 95 claim:—

1. The method of melting ferro-manganese, which consists in charging a cupola with successive layers of ferro-manganese and coke, and with an element capable of 100 neutralizing destructive chemical bases produced by the oxidation of the ferro-manganese tapping at frequent intervals, and replenishing the charge so as to keep the cupola at its capacity at all times.

2. A continuous method of melting ferro-manganese, which consists in charging a cupola with ferro-manganese and coke, and

105

- melting the charge while maintaining low blast pressure, in the presence of a neutralizing agent capable of producing a fluid slag, and tapping the cupola at regular intervals.
- 5 3. A continuous method of melting ferro-manganese, which consists in charging a cupola with ferro-manganese and coke and a flux capable of neutralizing destructive influences upon the lining, melting with the aid of a low blast pressure, and tapping at frequent intervals.
4. A continuous method of melting ferro-manganese in a cupola, which consists in charging the latter with ferro-manganese

and coke in excess of that required for the 15 day's run.

5. A continuous method of melting ferro-manganese in a cupola, which consists in charging the latter with ferro-manganese and coke in excess of that required for the 20 day's run, melting while maintaining a comparatively low blast pressure, and tapping at frequent intervals.

In testimony whereof we affix our signatures.

JOHN H. HALL.  
RICHARD D. JORDAN.